

L. HUSSON,  
PHOTOGRAPHIC DRY PLATE,  
APPLICATION FILED SEPT. 19, 1906.

922,908.

Patented May 25, 1909.

*Fig. 1.*



*Fig. 2.*



Witnesses  
P. F. Nagle.  
L. Donville.

Inventor  
Louis Husson  
By  
Nederhewitt & Fairbanks  
Attorneys

# UNITED STATES PATENT OFFICE.

LOUIS HUSSON, OF PHILADELPHIA, PENNSYLVANIA, ASSIGNOR OF ONE-HALF TO ANDRÉ F. BORNOT, OF PHILADELPHIA, PENNSYLVANIA.

## PHOTOGRAPHIC DRY-PLATE.

No. 922,908.

Specification of Letters Patent.

Patented May 25, 1909.

Application filed September 19, 1906. Serial No. 335,659.

*To all whom it may concern:*

Be it known that I, LOUIS HUSSON, a citizen of the United States, residing in the city and county of Philadelphia, State of Pennsylvania, have invented a new and useful 5 Photographic Dry-Plate, of which the following is a specification.

My invention relates to improvements in photographic dry plates adapted for printing 10 in different colors and its object is to render the plates more sensitive to particular colors with the addition of certain dye colors without the employment of color screen ray filters, as heretofore.

15 The invention consists in the employment of a repellent on the surface of a gelatin bromid plate whereby I am enabled to coat such plate with an extra value color without interfering with the working power of the 20 light in exposing such plate nor in any manner with the developing or tinting of the plate, the colors I employ being adapted to disappear with the regular working of the plates.

25 Figures 1 and 2 represent face views of opposite sides of plates that may be employed in carrying out my invention, and in which—

A designates a plate of glass or other suitable transparent material on which is a 30 sensitized coating B, which generally is of a very light blue color, C a repellent on said coating B, the same being colorless like water, and D a coating of coloring material, which may be red, green, etc., the same being 35 on the repellent, the latter serving to prevent admixture of the coatings B and D.

In carrying out my invention, I take a ready made gelatin bromid orthochromatic or isochromatic plate or any ordinary gelatin 40 bromid plate sensitive to one or several colors. I coat this plate first with a repellent made of wax, spermaceti, paraffin, stearic acid or the like dissolved in a volatile liquid such as a benzin, benzole, ether or the like.

45 The function of the repellent is to prevent the second color solution, to be applied later, from mixing with the gelatin bromid plate. When the coating is dry, I rub the plate with 50 cotton absorbent or chamois skin and thus polish the same.

The plate is now coated with a coloring solution appropriate to the deepness of the color desired on the plate, such solution being composed of coloring matter dissolved in alcohol, ether, acetone or other suitable volatile liquid with the addition of glucose or glycerin to increase the body thereof, the solution remaining on the surface of the absolutely dry plate producing two distinct 55 coatings, the resultant plate permitting a 60 perfect action of light therethrough and being adapted for making negatives of objects of all sorts for the three colored half tone process made on metal, for transfers on stone or for the collotype process. 65

The preferable color solution formula employed is as follows:—alcohol (95%) 1 dram, liquid glucose, 2 ounces, or glycerin 2 ounces, anilin colors (about) 6 gr. Mix at from 90° to 100° Fahrenheit. Then add 70 organic acid such as citric, acetic, formic acid or the like until blue litmus paper turns red. After having the repellent put on the plate as described coat the plate very evenly with the above solution and dry in gyrating 75 machine.

I am also enabled to shorten the exposure so as to make portraits practically from life with three, four or five different negatives.

Having thus described my invention, 80 what I claim as new and desire to secure by Letters Patent, is:—

1. A photographic plate having a plurality of coatings, a portion composed of a repellent and another portion composed of a coloring 85 solution.

2. A photographic plate coated with a repellent composed of wax, and a coloring solution composed of coloring matter dissolved in a volatile liquid. 90

3. A photographic plate coated with a repellent composed of wax, and a coloring solution composed of coloring matter dissolved in a volatile liquid and material to increase the body of the solution.

LOUIS HUSSON.

Witnesses:

JOHN A. WIEDERSHEIM,  
S. R. CARR.